

Dec. 27, 1932.

F. B. NIMICK

1,891,943

METHOD OF MAKING GROUND RODS

Filed July 22, 1931



*Fig. 1.*



*Fig. 2.*



*Fig. 3.*



INVENTOR

*Francis B. Nimick,  
By Archworth Martin,  
Attorney.*

## UNITED STATES PATENT OFFICE

FRANCIS B. NIMICK, OF CORAOPOLIS, PENNSYLVANIA, ASSIGNOR TO COLONIAL STEEL COMPANY, OF PITTSBURGH, PENNSYLVANIA, A CORPORATION OF PENNSYLVANIA

## METHOD OF MAKING GROUND RODS

Application filed July 22, 1931. Serial No. 552,403.

My invention relates more particularly to ground rods such as are employed in connection with electrical transmission lines, but is also susceptible of use in various other ways.

5 Ground rods frequently consist of bars which are driven into the ground to serve as anchoring posts and also as ground conductors. Conductor bars have heretofore been composed of a core or main body portion of 55 steel or the like and a sheath or sleeve of copper or other material, the steel being employed for the purpose of strength and the copper by reason of its conductivity and non-corrosive character, but such composite bars 10 have been commonly either square or round 15 in cross section.

One object of my invention is to provide a ground rod of the type referred to, which for a given cross sectional area, has relatively great surface area and hence greater conductivity than bars of the forms heretofore employed, and which also is possessed of greater mechanical strength.

Another object of my invention is to provide ground rods of generally improved characteristics in the way of form and efficiency.

In order to permit of the clear understanding of my invention, I have shown various features thereof in the accompanying drawing, wherein Figure 1 is a perspective view of my rod at a preliminary stage in the process of forming the same; Fig. 2 is a similar view showing another form of composite blank from which a completed ground rod 30 may be formed; Fig. 3 is an elevational perspective view of a feeder rod formed from a composite blank shaped according to either Fig. 1 or Fig. 2, and Fig. 4 is a cross sectional view of the rod of Fig. 3.

40 While I hereinafter describe a ground rod that is ribbed, it will be understood that the rod may be fluted, grooved, or otherwise shaped to provide an exposed surface that is relatively great, compared to the cross sectional area of the bar.

45 Referring to Fig. 1, a bar 4 of steel or the like, is covered by a copper sleeve or sheath 5, as by a welding operation well-known in the art, or by a combined welding and rolling or drawing operation. Again, the cop-

per may be electrically deposited upon the steel. In any case, I have a structure wherein the core or body portion 4 possesses great strength, as in the case of steel, which can be driven into the ground, and a structure 55 wherein the sheath 5 serves to effectively conduct electrical currents to the ground and to protect the bar 4 against corrosion, etc.

The blank of Fig. 1 is rolled or otherwise reshaped to form ribs thereon, or to flute the 60 same, in directions parallel to the longitudinal axis of the bar, and to give it an appearance similar to that shown in Figs. 3 and 4, so that while the bar contains the same amount of metal as in its original form, there 65 is, nevertheless, a greater area of the sheath 5 exposed than in the case of the structure of Fig. 1, thus providing for greater surface contact with the ground and better electrical conductivity. Furthermore, the longitudinal 70 ribs increase the mechanical strength of the bar as shown in Fig. 3, relative to the strength present in the bar of Fig. 1. This increased strength is particularly desirable, because the rod must frequently be driven 75 into hard ground, and furthermore it has increased resistance to transverse stresses.

The blank of Fig. 1 is heated to forging or rolling temperature to facilitate the rolling and shaping thereof as above-described.

The blank of Fig. 2 is shaped to the form shown in Figs. 3 and 4, by heating and rolling or otherwise shaping it, the end of the copper sleeve 5a being drawn to a point to completely enclose the end of the core bar 4a. 85 In other words, a rod formed from the blank of Fig. 2 will have the appearance of the rod shown in Figs. 3 and 4, with the copper completely enclosing the lower end of the core 90 bar 4.

A conductor wire 6 leading from a line or structure to be grounded is placed within one of the flutes of the bar, and may be securely maintained therein in any suitable manner as by coiling a wire snugly around 95 the ground rod and the ground wire, or by suitable clamping means such as an ordinary hose clamp.

The placing of the ground wire 6 in a groove provides an extended electrical con- 100

tact between it and the ground rod much greater than in those cases where the ground wire is simply secured against the side of a circular or flatside ground rod.

5 I claim as my invention:-

1. The method of making ground rods which comprises covering a hard metal bar with a close-fitting tubular sheath that is open at one end and is of more ductile metal

10 that has high electrical conductivity, heating the composite structure to forging temperature and shaping the composite structure to form ribs extending longitudinally thereof, and to cause said ductile metal to completely enclose the said end of the said bar.

15 2. The method of making ground rods which comprises covering a hard metal bar with a close-fitting tubular sheath that is open at one end and is of more ductile metal

20 that has high electrical conductivity, heating the composite structure to forging temperature and shaping the composite structure to form ribs extending longitudinally thereof, and to cause said ductile metal to completely enclose the said end of the said bar,

25 an additional forging operation being performed on said end to draw it to a point.

30 3. The method which comprises covering a hard metal bar with a close-fitting sheath

35 of more ductile metal, and which is open at one end, heating the composite structure to forging temperature, rolling the composite bar toward said end, to form ribs extending longitudinally thereof and to effect elongation

40 of the sheath relative to the bar, and compressing the said end of the composite bar to effect pointing thereof and cause the enclosure of the core point by the sheath.

45 4. The method which comprises covering a hard metal bar with a close-fitting sheath of more ductile metal and which is open at one end, rolling the composite bar toward said end to effect elongation thereof, and compressing said end of the composite bar to

50 effect pointing thereof and cause the enclosure of the core point by the sheath.

55 5. The method which comprises covering a cylindrical bar of relatively hard metal with a close-fitting cylindrical sheath of more ductile metal, heating the composite structure to forging temperature, applying radially

55 inward forging pressure to said bar from opposite sides thereof on two diametral lines disposed at right angles to one another, effecting elongation of the sheath relative to the bar, and compressing the composite structure near one end thereof to produce a point thereon and cause the enclosure of the core

60 point by the sheath.

65 In testimony whereof I, the said FRANCIS B. NIMICK, have hereunto set my hand.

FRANCIS B. NIMICK.